

## UNITED STATES PATENT OFFICE

2,640,053

## COMPOUNDED LUBRICATING OIL

Max W. Hill, Somerville, and Robert H. Jones, Kenilworth, N. J., assignors to Standard Oil Development Company, a corporation of Delaware

No Drawing. Application November 23, 1949,  
Serial No. 129,196

13 Claims. (Cl. 260—139)

1

This invention relates to mineral oil compositions and particularly to lubricants containing a detergent additive.

The art of metallic detergents for lubricating oil compositions adapted for use in internal combustion engines is well known to those versed in this field and has resulted in substantial improvements in lubricants. These detergents are particularly useful in lubricating oil compositions which are employed in internal combustion engines used in the operations of automobiles, aircraft and similar vehicles, including diesel engines, to improve their operation by preventing or retarding corrosion, piston ring sticking, cylinder wear, and carbon and varnish formation. However, when metallic detergents are used in lubricating compositions where oil consumption is high and engine conditions are severe, such as in aircraft engines or where such concentrations of metallic detergents are used to maintain engine cleanliness under conditions where high deposit fuels of cracked or high sulfur nature are used, such as in automobile and diesel operation, the ash content from the metallic detergent accumulates in the combustion chamber and causes pre-ignition, detonation, spark plug fouling, valve burning, and ultimate destruction of the engine.

It is known that the acidic product obtained by reacting a sulfide of phosphorus with a hydrocarbon possess mild detergent properties when incorporated in a mineral lubricating oil. However, this product is objectionable for commercial use in the fact that it gradually evolves hydrogen sulfide and accordingly gives forth a very disagreeable odor. Furthermore, such products are unstable and on standing for a short time at room temperature tend to precipitate a light colored solid material.

It has been found, in accordance with the present invention that if this reaction product of phosphorus sulfide and a hydrocarbon or essentially hydrocarbon material is contacted with a hydrocarbon having one or more olefinic double-bonds, a reaction takes place with the evolution of heat, even at ordinary temperatures; and the product of this reaction is not only very satisfactory from the standpoint of detergency and corrosion inhibiting properties when incorporated in lubricating oils and other mineral oil products, but also is more stable with respect to hydrogen sulfide evolution and precipitation of solids on standing for long periods of time. Furthermore, because the product contains no metal, it is free from the objectionable feature of leaving a metal-

lic deposit or ash when used as an additive for the crankcase lubricant of an internal combustion engine. These compounds are also effective, not only when added directly to the crankcase lubricant, but also when added to the engine fuel, since in the operation of the engine it will work its way from the combustion chamber into the crankcase and there blend with the lubricant.

In the first step of the preparation of the additives employed in accordance with the present invention a sulfide of phosphorus is reacted with a hydrocarbon material. The sulfide of phosphorus which can be employed includes  $P_2S_3$ ,  $P_2S_5$ ,  $P_4S_3$ ,  $P_4S_7$  or other phosphorus sulfide, and is preferably phosphorus pentasulfide ( $P_2S_5$ ). Mixtures of two or more phosphorus sulfides may also be employed as well as mixtures of elemental phosphorus and sulfur.

The hydrocarbon materials which may be reacted with a phosphorus sulfide may be paraffins, olefins, or olefin polymers, diolefins, acetylenes, aromatics or alkyl aromatics, cyclic aliphatics, petroleum fractions, such as lubricating oil fractions, petrolatums, waxes, cracked cycle stocks, or condensation products of petroleum fractions, solvent extracts of petroleum fractions, etc.

Essentially paraffinic hydrocarbons such as bright stock residuums, lubricating oil distillates, petrolatums or paraffin waxes may be employed. There may also be employed products obtained by condensing any of the foregoing hydrocarbons, usually through first halogenating the hydrocarbon, with aromatic hydrocarbons in the presence of anhydrous inorganic halides, such as aluminum chloride, zinc chloride, boron fluoride, and the like.

As examples of monoolefins may be mentioned isobutylene, acrolein, decene, dodecene, cetene ( $C_{16}$ ), octadecene ( $C_{18}$ ), cerotene ( $C_{28}$ ), melene ( $C_{30}$ ), olefinic extracts from gasoline or gasoline itself, cracked cycle stocks and polymers thereof, resin oils from crude oil, hydrocarbon coil resins, cracked waxes, dehydrohalogenated chlorinated waxes, and any mixed high molecular weight alkenes obtained by cracking petroleum oils. A preferred class of olefins are those having at least 20 carbon atoms per molecule, of which from about 12 to about 18 carbon atoms, and preferably at least 15 carbon atoms, are in a long chain. Such olefins may be obtained by the dehydrogenation of paraffin waxes, by the dehydrohalogenation of long chain alkyl halides, by the synthesis of hydrocarbons from  $CO$  and  $H_2$ , by the dehydration of alcohols, etc.

Another class of suitable olefinic materials are

the monoolefin polymers, in which the molecular weight ranges from 100 to 50,000, preferably from about 250 to about 10,000. These polymers may be obtained by the polymerization of low molecular weight monoolefinic hydrocarbons, such as ethylene, propylene, butylene, isobutylene, normal and isoamylanes, or hexenes, or by the copolymerization of any combination of the above monoolefinic materials.

Diolefins which may be employed include well known materials such as butadiene, isoprene, chloroprene, cyclopentadiene, 2,3-dimethylbutadiene, pentadiene-1,3, hexadiene-2,4, terpenes, and the like. Acetylene and substituted acetylenes may similarly be employed.

Another class of unsaturated hydrocarbon materials which may be advantageously employed in the preparation of the additives of this invention are high molecular weight copolymers of low molecular weight monoolefins and diolefins. The copolymer is prepared by controlled copolymerization of a low molecular weight olefin and a non-aromatic hydrocarbon showing the general formula  $C_nH_{2n-x}$ , in which  $x$  is 2 or a multiple of 2, in the presence of a catalyst of the Friedel-Crafts or peroxide type. The low molecular weight olefin is preferably an isoolefin or a tertiary base olefin preferably one having less than 7 carbon atoms per molecule. Examples of such olefins are isobutylene, 2-methylbutene-1,2-ethylbutene-1, secondary and tertiary base amylene, hexylenes, and the like. Examples of the non-aromatic hydrocarbons of the above formula which can be used are the conjugated diolefins listed in the preceding paragraph, diolefins such as 1,4-hexadiene, in which the double bond is not conjugated, as well as the acetylenes. The copolymerization is preferably carried out in the presence of aluminum chloride, boron fluoride, or benzoyl peroxide, and the copolymer is preferably one having a molecular weight of about 1,000 to 30,000.

Another class of hydrocarbons which may be employed in a similar manner are aromatic hydrocarbons, such as benzene, naphthalene, anthracene, toluene, xylene, diphenyl, and the like, as well as aromatic hydrocarbons having alkyl substituents and aliphatic hydrocarbons having aryl substituents.

A still further class of hydrocarbons which may be employed in the reaction with sulfides of phosphorus are condensation products of halogenated aliphatic hydrocarbons with an aromatic compound, produced by condensation in the presence of aluminum chloride or other Friedel-Crafts type catalyst. The halogenated aliphatic hydrocarbon is preferably a halogenated long chain paraffin hydrocarbon having more than 8 carbon atoms, such as paraffin wax, petrolatum, ozocerate wax, etc. High viscosity paraffin oils, particularly heavy residual oil which has been treated with chemicals or extracted with propane or other solvents for the removal of asphalts, may be employed. The aromatic constituent may be naphthalene, fluorene, phenanthrene, anthracene, coal tar residues, and the like.

Another type of hydrocarbon material which may be similarly employed is a resin-like oil which has a molecular weight of from about 1,000 to 2,000 or higher, obtained preferably from a paraffinic oil which has been dewaxed and which is then treated with a liquified normally gaseous hydrocarbon, e. g., propane, to precipitate a heavy propane-insoluble fraction. The latter is a substantially wax-free and asphalt-free product

having a Saybolt viscosity at 210° F. of about 1,000 to about 4,000 seconds or more.

The phosphorus sulfide-hydrocarbon reaction product may be readily obtained by reacting the phosphorus sulfide with the hydrocarbon at a temperature of about 200° F. to about 600° F., and preferably from about 300° F. to about 550° F., using from about one to about ten, preferably about two to about five molecular proportions of hydrocarbon to one molecular proportion of the sulfide of phosphorus in the reaction. It is advantageous to maintain a non-oxidizing atmosphere, such as an atmosphere of nitrogen, above the reaction mixture. Usually it is desirable to use an amount of the phosphorus sulfide that will completely react with the hydrocarbon so that no further purification becomes necessary. In the case of monoolefin polymers the preferred ratio is one molecular proportion of the sulfide of phosphorus to two to five molecular proportions of polymer. In such case the reaction is continued until all or substantially all of the phosphorus sulfide has reacted. The reaction time is not critical, and the time required to cause the maximum amount of phosphorus sulfide to react will vary with the temperature. A reaction time of two to ten hours is frequently necessary. If desired, the reaction product may be further treated by blowing with steam, alcohol, ammonia, or an amine at an elevated temperature of about 200° F. to about 600° F. to improve the odor thereof.

The product obtained by reacting a sulfide of phosphorus with a hydrocarbon material in accordance with the process described above is then further reacted with an unsaturated hydrocarbon by contacting the two materials at room temperature, if desired, or more preferably at a somewhat elevated temperature of the order of 150-380° F., using from about 0.1% to 50%, preferably about 5% to 20%, by weight of the unsaturated hydrocarbon, based on the amount of phosphorus sulfide-hydrocarbon product present.

The reaction is continued for a period of about one to about ten hours. The unreacted olefin is removed from the final product by distillation. However, in certain instances it may be desirable to employ an excess of the olefinic material or other unsaturated hydrocarbon products, then adding a sufficient quantity of sulfur to form a still more effective addition agent. This last step may also be made more effective by the addition of an agent commonly used in the vulcanization of rubber, such as Tuads, Captax, Tellurac, Selenac, or guanidine or substituted guanidines.

The unsaturated hydrocarbon material which is reacted with the phosphorus sulfide-hydrocarbon product in accordance with the present invention may be any aliphatic, cycloaliphatic, terpenic, or aliphatic-aromatic hydrocarbon containing at least one double bond carbon-to-carbon linkage in a non-aromatic group. The materials more preferably employed include the olefins, e. g., propylenes, butylenes, diisobutylenes, triisobutylenes, the codimer of isobutylene and n-butylene, also cracked gasoline fractions, cracked paraffin wax, viscous olefin polymers such as medium or high molecular weight polybutene, cyclopentene, cyclohexene, butadiene, pentadiene, isoprene, dipentene,  $\alpha$ -pinene,  $\beta$ -pinene, terpinolene,  $\Delta 2,4(8)$ -p-menthadiene, styrene, and the like. Derivatives of the above described compounds containing various non-reactive substituent groups and atoms may be used to advantage, since such groups or

atoms would not interfere with the reaction. Such substituted groups and atoms include nitro groups, halogen atoms, etc. Hydrocarbon materials containing from 2 to 30 carbon atoms per molecule may generally be employed.

Since the additives of the present invention are to be dissolved in mineral oils, the hydrocarbons which are reacted with a sulfide of phosphorus, and the materials which are further reacted with the products thus formed will be chosen with a view to provide a product which is soluble in the oil base or which has such marginal solubility that it can be plasticized with a high molecular weight alcohol, esters, or other plasticizer.

When additives of the present invention are employed in mineral lubricating oils, they are preferably added in proportions of about 0.001 to about 10.0% and preferably 1.0 to about 6.0%. The proportions giving the best results will vary somewhat according to the nature of the additive and the specific purpose which the lubricant is to serve in a given case. For commercial purposes, it is convenient to prepare concentrated oil solutions in which the amount of additive in the composition ranges from 25% to 50% by weight, and to transport and store them in such form. In preparing a lubricating oil composition for use as a crankcase lubricant the additive concentrate is merely blended with the base oil in the required amount.

In certain cases it may be found that the effect of adding compounds of the type described above to a lubricating oil will be to increase the detergent effect of the oil without sufficiently providing oxidation resisting characteristics. In such a case it is advantageous to add to the lubricant, in addition to the additives of the present invention, a substance containing sulfur and/or phosphorus. Elemental sulfur may be used for this purpose or an organic sulfur compound, particularly an organic sulfur compound capable of being decomposed to give free sulfur at a temperature to which the lubricant is subjected during use. Examples of such organic sulfur compounds are sulfurized mineral oils, terpenes, olefins, and diolefins, sulfurized animal and vegetable oils, sulfurized isobutylene polymer, etc.

Below are given detailed descriptions of preparations of examples of lubricating oil additives described above as well as engine tests in which an oil containing the additives was used as the lubricant. It is to be understood that these examples are given as illustrations of the present invention and are not to be construed as limiting the scope thereof in any way.

*Example 1*

42.4 lbs. of a lubricating oil bright stock of 150 seconds viscosity (Saybolt) at 210° F. was treated with 10 g. of benzoyl peroxide and 4.25 lbs. of P<sub>2</sub>S<sub>5</sub>. The mixture was stirred under an atmosphere of nitrogen gas at 350-370° F. for 3 hours and filtered. 250 g. of the product thus obtained and 25 g. of diisobutylene were vigorously stirred and heated for two hours at 240-260° F. Nitrogen gas was bubbled through the reaction mixture and the temperature was raised to about 400° F. over a two hour period and the finished additive obtained by filtration.

*Example 2*

A product was obtained using the same reaction conditions and the same materials as in Example

1, except that commercial dipentene<sup>1</sup> was used instead of diisobutylene in the second step of the process.

*Example 3.—Lauson engine test*

The products prepared by the methods of Examples 1 and 2 and a sample of the untreated P<sub>2</sub>S<sub>5</sub>-bright stock reaction product were blended in 4% concentration in a lubricating oil base consisting of a solvent extracted Coastal naphthenic oil of 60 seconds (Saybolt) viscosity at 210° F. The blends were submitted to a standard Lauson engine test, which was conducted by operating the Lauson engine at 1800 R. P. M. for 20 hours with a 1.5 indicated kilowatt load, 300° F. oil temperature and 295° F. water jacket temperature. A similar test was applied to the unblended base oil. The oils were rated by the demerit system, wherein an oil which produces a perfectly clean piston surface is given a rating of zero, while a rating of 10 is given to an oil which produces the worst condition which could be expected on that surface. The loss in weight of the copper-lead bearing was also determined. The results are shown in the following table:

|    | Oil Composition                                                           | Piston Skirt<br>Varnish<br>Demerit | Cu-Pb Bear-<br>ing Wt. Loss<br>(g./bearing) |
|----|---------------------------------------------------------------------------|------------------------------------|---------------------------------------------|
| 30 | Base oil                                                                  | 4.50                               | 0.10                                        |
|    | Base oil+4% untreated P <sub>2</sub> S <sub>5</sub> -bright stock product | 2.25                               | 0.02                                        |
|    | Base oil+4% product of Example 1                                          | 1.75                               | 0.01                                        |
|    | Base oil+4% product of Example 2                                          | 0.38                               | 0.03                                        |

The products of the present invention may be employed not only in ordinary hydrocarbon lubricating oils but also in the "heavy duty" type of lubricating oils which have been compounded with such detergent type additives as metal soaps, metal petroleum sulfonates, metal phenates, metal alcoholates, metal alkyl phenol sulfides, metal organo phosphates, phosphites, thiophosphates, and thiophosphites, metal xanthates and thioxanthates, metal thiocarbamates, and the like. Other types of additives, such as phenols and phenol sulfides, may also be present.

The lubricating oil base stock used in the compositions of this invention may be straight mineral lubricating oils or distillates derived from paraffinic, naphthenic, asphaltic or mixed base crudes, or, if desired, various blended oils may be employed as well as residuals, particularly those from which asphaltic constituents have been carefully removed. The oils may be refined by conventional methods using acid, alkali and/or clay or other agents such as aluminum chloride, or they may be extracted oils produced by solvent extraction with solvents such as phenol, sulfur dioxide, etc. Hydrogenated oils or white oils may be employed as well as synthetic oils prepared, for example, by the polymerization of olefins or by the reaction of oxides of carbon with hydrogen or by the hydrogenation of coal or its products. In certain instances cracking coal tar fractions and coal tar or shale oil distillates may also be used. Also, for special applications, animal, vegetable or fish oils or their hydrogenated or volatized products may be employed in admixtures with mineral oils.

For the best results the base stock chosen should normally be an oil which with the new additive present gives the optimum performance

<sup>1</sup> The commercial "dipentene" employed had the following composition: dipentene—31%, terpinolene—39%, α-pinene—6%, α-terpineol—7%, Δ<sub>2,4(8)</sub>-p-menthadiene—5%, para-cymene—10%, residue—2%.

in the service contemplated. However, since one advantage of the additives is that their use also makes feasible the employment of less satisfactory mineral oils, no strict rule can be laid down for the choice of the base stock. The additives are normally sufficiently soluble in the base stock, but in some cases auxiliary solvent agents may be used. The lubricating oils will usually range from about 40 to 150 seconds (Saybolt) viscosity at 210° F. The viscosity index may range from 0 to 100 or even higher.

Other agents than those which have been mentioned may be present in the oil composition, such as dyes, pour point depressants, heat thickened fatty oils, sulfurized fatty oils, sludge dispersers, antioxidants, thickeners, viscosity index improvers, oiliness agents, resins, rubber, olefin polymers, and the like.

Assisting agents which are particularly desirable as plasticizers and defoamers are the higher alcohols having preferably 8-20 carbon atoms, e. g. octyl alcohol, lauryl alcohol, stearyl alcohol, and the like.

In addition to being employed in lubricants, the additives of the present invention may also be used in other mineral oil products such as motor fuels, hydraulic fluids, torque converter fluids, cutting oils, flushing oils, turbine oils, transformer oils, industrial oils, process oils, and the like, and generally as antioxidants in mineral oil products. They may also be used in gear lubricants, greases and other products containing mineral oils as ingredients.

Since the reaction products of the present invention are powerful surface acting agents, they have practical use in dry cleaning fluids, in mineral spirit and aqueous paints, as flotation agents, as dispersants for insecticides in aqueous and non-aqueous solutions, and as additives for natural and synthetic rubber, as carbon black dispersants, and as vulcanization accelerators. The products of this invention may also be used as metal dispersants and antioxidants in colloidal iron electromagnetic clutches. They are useful dispersants in printing ink, asphalts, linoleum, roofing compositions, drilling muds, metal cleaners and pickling solutions, and as general commercial dispersant aids.

What is claimed is:

1. As a new composition of matter a product obtained by reacting about one molecular proportion of a phosphorus sulfide with two to five molecular proportions of a hydrocarbon and further reacting the acidic product thus formed with 0.1% to 50% of its weight of a hydrocarbon containing at least one olefinic double bond.

2. As a new composition of matter a product according to claim 1 in which the sulfide of phosphorus is phosphorus pentasulfide.

3. As a new composition of matter a product according to claim 1 in which the sulfide of phosphorus is phosphorus pentasulfide and in which the hydrocarbon material reacted with the same is a lubricating oil bright stock.

4. As a new composition of matter a product according to claim 3 in which the P<sub>2</sub>S<sub>5</sub>-bright stock product is reacted with diisobutylene.

5. As a new composition of matter a product according to claim 3 in which the P<sub>2</sub>S<sub>5</sub>-bright stock product is reacted with a terpene.

6. The method which comprises reacting one molecular proportion of a sulfide of phosphorus

with two to five molecular proportions of a hydrocarbon and further reacting the product thus formed with a hydrocarbon containing at least one olefinic double bond.

5 7. A method according to claim 6 in which the phosphorus-sulfide-hydrocarbon reaction product is contacted with the unsaturated hydrocarbon at a temperature ranging from room temperature to 380° F.

10 8. The method which comprises reacting one part by weight of phosphorus pentasulfide with ten parts by weight of a lubricating oil bright stock at a temperature of about 350-370° F. for 3 hours, and further treating ten parts by weight of the product thus formed with one part by weight of diisobutylene at 240°-260° F. for a period of two hours and further heating the reaction mixture at a temperature of about 400° F. for an additional two hour period.

20 9. A method which comprises treating one part by weight of phosphorus pentasulfide with ten parts by weight of a lubricating oil bright stock for a period of three hours at 350-370° F., and further treating ten parts by weight of the product thus formed with about one part by weight of a terpene for a period of two hours at 240-260° F. and for an additional period of two hours at a temperature of about 400° F.

10 10. As a new composition of matter, a product obtained by reacting from one to about 10 molecular proportions of a hydrocarbon with one molecular proportion of a sulfide of phosphorus at a temperature above about 200° F. and further reacting the phosphorus- and sulfur-containing material so formed with from 0.1 to 50% of its weight of an olefinic hydrocarbon containing at least one olefinic double bond whereby a product of improved stability is formed.

11 11. A composition according to claim 10 in which said phosphorus- and sulfur-containing material is reacted with from 5 to 20 weight per cent of said olefinic hydrocarbon.

12 12. A composition according to claim 10 in which said olefinic hydrocarbon is selected from the group consisting of aliphatic, cycloaliphatic, terpene and aliphatic-aromatic mono-olefins and di-olefins.

13 13. A process for producing a substantially stable phosphorus- and sulfur-containing hydrocarbon which comprises the steps of reacting from one to about 10 molecular proportions of a hydrocarbon with one molecular proportion of a sulfide of phosphorus at a temperature of from about 200° F. to 600° F. for at least two hours, and further reacting the resulting product with an amount of an olefinic hydrocarbon at a temperature of from room temperature to about 380° F. sufficient to form a product having improved stability characteristics.

60

MAX W. HILL.  
ROBERT H. JONES.

References Cited in the file of this patent

UNITED STATES PATENTS

| Number    | Name    | Date          |
|-----------|---------|---------------|
| 2,315,529 | Kelso   | Apr. 6, 1943  |
| 2,356,073 | May     | Aug. 15, 1944 |
| 2,379,312 | May     | June 26, 1945 |
| 2,413,648 | Ott     | Dec. 31, 1946 |
| 2,483,600 | Stucker | Oct. 4, 1949  |
| 2,507,731 | Mixon   | May 16, 1950  |